

A. RIDD.

PROCESS OF FINISHING METAL SHEETS OR PLATES.

APPLICATION FILED DEC. 22, 1913.

1,133,670.

Patented Mar. 30, 1915.



*Fig. 1.*



*Fig. 2.*

Witnesses

*J. P. Jones  
S. Willow.*

*A. Ridd,*

Inventor

by *C. A. Moore Co.*  
Attorneys

# UNITED STATES PATENT OFFICE.

AMBROSE RIDD, OF BRACKENRIDGE, PENNSYLVANIA.

## PROCESS OF FINISHING METAL SHEETS OR PLATES.

1,133,670.

Specification of Letters Patent Patented Mar. 30, 1915.

Application filed December 22, 1913. Serial No. 808,244.

To all whom it may concern:

Be it known that I, AMBROSE RIDD, a citizen of the United States, residing at Brackenridge, in the county of Allegheny and State of Pennsylvania, have invented a Process of Finishing Metal Sheets or Plates, of which the following is a specification.

The present invention relates to an improved process of finishing metal sheets or plates, whereby an even oxidization or bluing is given the surfaces thereof.

Heretofore many processes have been devised to accomplish the even oxidization or bluing of the metal sheets or plates, the better ones of which consist in placing the sheets or plates in an annealing box and subjecting them to an annealing degree of heat without contact with the atmospheric air, the top or cover of the annealing box being removed and the sheets or plates being then removed, some being rolled in the presence of atmospheric air and others being exposed for oxidization and then subjected to heat above the degree to which they have fallen. Both of these processes have their faults, in that the edges of the plates are too greatly discolored, while the lowermost plates often have to be again placed through the process.

In carrying out the present process, the metal sheets or plates are placed in an annealing box, and there subjected to an annealing degree of heat without contact with the air, and when they are at a lower temperature, or at a cherry red heat, the cover of the annealing box is removed and the sheets or plates are placed in a heated box and sealed, and then subjected to a heat that maintains them at the cherry red heat, and out of contact with the atmospheric air. After a period of such subjection, the sheets or plates are removed singly or in packs, from the latter box without removing its cover and during such removal, are exposed to the atmospheric air. By doing this, each sheet has the same exposure and an even oxidization or coloring is given each and every sheet.

In carrying out the present invention, one form of apparatus is here illustrated and set forth in the accompanying drawings, in which—

Figure 1 is a view in section of an annealing oven which contains the sheets to be annealed therein and which may be rolled or moved into the annealing furnace. Fig. 2 represents in section the heat retaining re-

ceptacle where the annealed sheets are stored prior to the exposing of the same to the atmosphere.

Referring to the drawings in which similar reference numerals designate corresponding parts throughout the several views, the annealing oven includes the car 3 and the cover 4, the latter being provided with suitable lugs or equivalents 5 so that the cover may be readily removed from the car or placed thereupon. The car 3 with the cover 4 constitutes an annealing oven which may be rolled into or out of an annealing furnace so that the contents of the oven will be heated to a high temperature and allowed to cool out of contact with the atmosphere, which is secured by the placing of sand or other material 6 around the junction between the cover and car. 75

A table 7 is positioned upon the car 3 and upon which are stacked the sheets 8 which are to be annealed and blued. The car with the cover placed thereon and sealed thereto and with the sheets 8 arranged upon the table 7 is placed within the oven, the oven is rolled into the annealing furnace (not shown) and is heated to the proper temperature, after which it is moved and allowed to cool to a temperature suitable for the exposing of the annealed sheets to the atmosphere so that a proper blue color and oxidation will be formed thereon. 85

It has been found in practice that if after the annealing oven has dropped to the desired temperature the cover 4 be removed and the sheets removed one at a time to thus expose the same to the atmosphere for the oxidation and bluing thereof, that the lowermost sheets will gradually cool and will oxidize around their exposed edges so that a uniform bluing and oxidation of the sheets toward the bottom of the pile cannot be obtained and which requires that a large number of the sheets be returned to the annealing furnace. 100

In order to overcome these objections, I provide a heat retaining receptacle which includes a suitable foundation or body portion 9 through which extend the flues 10. 105 The foundation or body portion 9 is formed of fire bricks upon the top of which is placed the plate 11 with the upturned rim 12 extending therearound. The front of the plate is provided with the sill or ledge 13. 110

Mounted upon the plate or top 11 is the

cover 14 which, similar to the cover 4 is provided with lugs or other means 15 whereby said cover may be engaged in order that it may be removed from or placed upon the plate 11. The cover is provided with the sliding door 16 in its front portion and which is guided in its movement by the side walls of the cover (not shown) and the door is limited to a lowermost position as illustrated in Fig. 2, by suitable stops arranged upon the sides of the door (not shown) so that as the cover is removed, the door 16 will not become detached therefrom. In this connection it is mentioned that the door is provided with the eye 17 to which is secured a suitable cable 18 whereby the door may be raised and lowered although it will be understood that other means may be used for the manipulation and control of the door. The rear end of the cover is also provided with the door 19 which slides over and is adapted to close the opening 20. A conveyer 21 of the usual type terminates adjacent the rear door opening 20 and provides a conveyer for the sheets as they are passed through the opening 20. Thus it will be apparent that the sheets may be removed through the door 16 located at the front of the sheet retaining receptacle or may be passed through the rear opening 20 and onto the conveyer 21.

The table 7 with the sheets 8 disposed thereon and while in a heated condition are removed from the annealing oven and placed within the heat retaining receptacle, it being noted that, the covers of the oven and receptacle are previously removed. The table 7 with its sheets 8 while in a heated condition are thus placed within a heat retaining receptacle as illustrated in Fig. 2. The heat retaining receptacle has been previously heated by the introducing and burning of suitable gases through the flues 10 and the heat retaining receptacle will thus be retained at the desired temperature and which will normally be at about a cherry red heat. After the table 7 and the annealed sheets 8 have been introduced within the heat retaining receptacle, a suitable non-oxidizing gas is introduced into the same through the flues 10 so that the sheets will be maintained at the desired temperature and out of contact with the air. The non-oxidizing gas may be previously heated so as to maintain the proper temperature within the heat retaining receptacle. The temperature of the heat retaining receptacle may be adjusted by introducing heated and burnt gases through the flues 10 as it is thought will be readily appreciated. The door 16 is then raised and the sheets removed from the receptacle or they may be passed out of the rear opening 20 onto the conveyer 21 and delivered to some required and distant point, with the result that the sheets will be exposed to the

atmosphere while heated at the proper temperature to thereby produce a uniform oxidation and coloring. Thus the sheets may be annealed and blued in bulk and each sheet will be oxidized and blued in a uniform manner and without requiring that any of the sheets be returned to the oven for a retreatment.

Having thus fully described my invention, what I claim is:

1. The process herein described of preparing metal sheets or plates, which consists in subjecting said sheets or plates to an annealing heat, reducing said heat, checking the reduction at an intermediate degree, 80 maintaining the heat at said intermediate degree in a non-oxidizing atmosphere, subjecting the plates to a heated non-oxidizing fluid while maintained at such intermediate degree, and finally exposing the sheets or 85 plates uniformly throughout their surfaces to an oxidizing agent.

2. The process herein described of preparing metal sheets or plates, which consists in subjecting said sheets or plates to an annealing heat, reducing said heat, checking the reduction at an intermediate degree, 90 maintaining the heat at said intermediate degree in a non-oxidizing atmosphere, subjecting the plates to a heated non-oxidizing 95 fluid while maintained at such intermediate degree, and finally exposing the sheets or plates uniformly to the surrounding atmosphere for oxidizing.

3. The process herein described of preparing metal sheets or plates, which consists in subjecting said sheets or plates to an annealing degree of heat and out of contact with the atmospheric air, subjecting said sheets or plates to a lower degree of heat 105 and out of contact with the atmospheric air and simultaneously to a heated non-oxidizing fluid, and finally subjecting said sheets or plates to the atmospheric air to produce an even oxidization of the surfaces.

4. The process herein described of preparing metal sheets or plates, which consists in placing the sheets or plates in an annealing box and subjecting them to an annealing degree of heat without contact with the atmospheric air, removing the sheets or plates in bulk and placing them in a heat retaining receptacle which has been previously heated at a lower degree than for annealing, said second receptacle maintaining the sheets or plates out of contact with the atmospheric air, removing the sheets or plates from the last receptacle and exposing them to the atmospheric air for oxidization.

5. The process herein described of preparing metal sheets or plates, which consists in subjecting the sheets or plates contained within an annealing box to an annealing furnace, withdrawing the box and sheets when red hot, removing the sheets or plates 130

and placing them in a previously heated second box, said second box having been heated to approximately the heat of the plates when removed from the annealing furnace, the sheets or plates being retained therein and out of contact with the atmospheric air, introducing a heated non-oxidizing fluid and removing the sheets or plates and exposing them to the air to oxidize them.

6. The process herein described of preparing metal sheets or plates which consists in subjecting the sheets or plates contained within an annealing box to an annealing furnace, withdrawing the box and sheets when red hot, removing the sheets or plates and placing them in a previously heated second box, said second box having been heated to approximately the heat of the plates when removed from the annealing furnace, the sheets or plates being retained therein and out of contact with the atmos-

pheric air, and removing the sheets or plates and exposing the same to atmospheric air.

7. The process herein described of preparing metal sheets or plates, which consists in subjecting the sheets or metal plates while contained in an annealing box to an annealing furnace, withdrawing the same when heated red hot, removing the sheets or plates and placing them within a previously heated second box, sealing the second box, and forcing a heated non-oxidizing fluid into the second box, and removing the sheets or plates from the second box and exposing the same to the atmospheric air.

In testimony that I claim the foregoing as my own, I have hereto affixed my signature in the presence of two witnesses.

AMBROSE RIDD.

Witnesses:

OMAR C. CRAIG,  
LYDA M. WATSON.